

## UNITED STATES PATENT OFFICE

2,096,976

## PAPER TOWEL

George A. Richter and Milton O. Schur, Berlin,  
N. H., assignors to Brown Company, Berlin,  
N. H., a corporation of Maine

No Drawing. Application December 12, 1931,  
Serial No. 580,734

4 Claims. (Cl. 92—68)

Among the important characteristics desired in a paper towel, may be mentioned absorbency, high wet as well as dry strength, softness, absence of removable fuzz or lint, and freedom from unpleasant odors. In other words, a paper towel should be of such character that it will rapidly absorb moisture from the skin of the user, without leaving upon the skin a fuzz of short fiber, and will be capable of being rubbed and manipulated during the drying of the skin without tearing, as well as being withdrawn from towel cabinets without tearing even when the hands of the prospective user are wet. These desiderata are realized only to a limited extent by the usual waterleaf paper towels now on the market, made up from the various kinds of wood pulp, including ground-wood pulp and chemical wood pulp, such as kraft and sulphite. The fault with these customary towels of commerce lies in the fact that in attaining such qualities as softness and absorbency, substantially unbeaten pulp is used as a raw material, which pulp leads to a paper having comparatively poor strength, especially wet strength, and tear resistance, although having a relatively high degree of absorbency.

In accordance with the present invention, we produce a paper towel which, like the towels heretofore made, is substantially free from non-cellulosic sizing material but which contains sufficient cellulose hydrate or gelatinized cellulose to impart thereto a wet strength vastly greater than that of a similar waterleaf towel. At the same time, we preserve the water-holding capacity of our towel at a value not much less than that of a similar waterleaf towel. In speaking of a "waterleaf towel", we mean a paper towel as heretofore produced, namely, one lacking not only non-cellulosic sizing material, but also any noteworthy amount of cellulose hydrate. In speaking of cellulose hydrate, we mean cellulose fibers which have been hydrated by prolonged beating, which is a mechanical operation, and/or by the employment of a suitable chemical which can be removed by washing so as to leave with the fibers no chemical which would have a deleterious effect on the skin of the towel user. The expression "cellulose hydrate", as we use it in the specification and in the claims, is not intended to embrace so-called regenerated cellulose, that is, cellulose which is derived from a cellulose derivative of the character of the xanthate, nitrate, or the like. We have found that we are able to secure the best qualities of softness, absorbency, and high wet and dry strengths by introducing as a more or less continuous phase into a waterleaf paper web sufficient cellulose hydrate or gelatinized cellulose to increase its wet strength markedly, and then mechanically breaking up the phase to enhance the softness and absorbency of the web while still maintaining its wet strength con-

siderably in excess of the wet strength of a similar waterleaf web. By carrying out a suitable mechanical manipulation on the web, the hardened cellulose hydrate can be broken up, not only on the surfaces of the web, but throughout the web, and be absorbed thereby. The mechanical manipulation may be effected in a variety of ways, as by drawing the web at an acute angle over a knife edge or in a tortuous path past a series of knife edges in tight frictional contact with the web. Or the web may undergo the disrupting action of a sand-roll or a sand-blast, or be subjected to a suitable creping or crimping operation.

Rather than using a single lot of pulp as the raw material and beating it to generate the appropriate amount of mechanically hydrated cellulose therein, it is possible, and indeed preferable, to use a batch of pulp in substantially unbeaten condition and to blend therewith in suitable amount another batch of thoroughly hydrated or gelatinized pulp, such as serves in the manufacture of so-called glassine papers. The latter procedure has the advantage that the batch of substantially unbeaten pulp being made up of fiber units of practically original length conduces to a towel web of improved physical characteristics, especially improved tear resistance. The gelatinized pulp should be added to the ungelatinized pulp in controlled amount, since otherwise the mixture might yield an unsatisfactory sheet, for instance, a sheet whose water absorbency is too low for toweling. We present herewith a table showing the increase in wet strength effected in paper sheets through the addition of various percentages of mechanically gelatinized pulp to a batch of substantially unbeaten kraft pulp. The gelatinized pulp was also prepared from kraft pulp as the raw material. The sheets were handmade, and hence had comparatively smooth surfaces.

| Percent<br>gelatinized<br>pulp in<br>mixture | Wet tensile<br>strength of<br>sheets |
|----------------------------------------------|--------------------------------------|
| 0                                            | .34                                  |
| 10                                           | .36                                  |
| 20                                           | .43                                  |
| 30                                           | .50                                  |
| 50                                           | .67                                  |

45

50

55

60

It is to be observed that the gelatinized pulp markedly increased the wet strength of the sheets, and that a mixture containing 50% gelatinized pulp yielded a sheet having a wet strength almost twice as great as that prepared from a pulp composed entirely of substantially unhydrated fibers. While the sheets containing the gelatinized cellulose were less absorbent than the

sheet lacking this material, nevertheless a sheet containing even as much as 50% gelatinized cellulose can well take up 200% by weight of water and can be subjected to creping or other mechanical manipulation designed to enhance its water absorbency materially. Such mechanical manipulation can be carried out to appreciate water absorbency greatly, while still maintaining the wet strength of the sheet considerably above that of a sheet composed entirely of substantially unhydrated pulp.

In making a toweling web containing chemically hydrated cellulose, even better results can be had than through the use of mechanically hydrated cellulose. Thus, we can start with a pre-fabricated, waterleaf web of paper composed entirely of substantially unbeaten pulp, that is, the ordinary paper toweling, pass the web through a bath of chemical hydrating agent under conditions designed to produce the proper amount of cellulose hydrate, then wash the web free of chemical hydrating agent, and finally dry it. Before or after drying, the web may be creped or otherwise mechanically treated to increase its softness and absorbency. Specifically, the waterleaf web can be immersed for a few seconds in nitric acid of 1.42 specific gravity at room temperature, then washed free of acid, and dried. We have found that the finished web not only has a wet strength many times that of the starting web, but that the increase in wet strength has been brought about with but little loss in water-holding capacity of the web, that is, while keeping its water-holding capacity substantially unimpaired, as hereinafter stated. Similar results may be obtained by treating the starting web with dilute formaldehyde solutions, then immersing the web in 72% sulphuric acid at room temperature, washing, and drying. Other hydrating agents, like zinc chloride and potassium thiocyanate, may be used in such a way as to hydrate or gelatinize the web just far enough to impart the desired wet strength thereto while keeping its water-holding capacity substantially unimpaired.

What we claim is:

1. A process which comprises treating an absorptive paper web consisting substantially entirely of cellulose with formaldehyde solution, then treating the web with a strong solution of mineral acid for a period of time controlled to permit such acid to hydrate the cellulose and thereby increase markedly the wet-strength of the web while its water-holding capacity is preserved substantially unimpaired, washing the web, and drying it. 5

2. A process which comprises treating an absorptive paper web consisting substantially entirely of cellulose with formaldehyde solution, then treating the web with a strong solution of mineral acid at room temperature for a period of time controlled to permit such acid to hydrate the cellulose and thereby increase markedly the wet-strength of the web while its water-holding capacity is preserved substantially unimpaired, washing the web, and subjecting the washed web 15 to a creping operation.

3. A process which comprises treating an absorptive paper web consisting substantially entirely of cellulose with dilute formaldehyde solution, then immersing the web in sulphuric acid 25 solution of a strength in the order of magnitude of about 72% for a period of time controlled to permit such acid to hydrate the cellulose and thereby increase markedly the wet-strength of the web while its water-holding capacity is preserved substantially unimpaired, washing the web, and drying it. 30

4. A process which comprises treating an absorptive paper web consisting substantially entirely of cellulose with dilute formaldehyde solution, then immersing the web in sulphuric acid 35 solution of a strength in the order of magnitude of about 72% and at room temperature for a period of time controlled to permit such acid to hydrate the cellulose and thereby increase 40 markedly the wet-strength of the web while its water-holding capacity is preserved substantially unimpaired, washing the web, and subjecting the washed web to a creping operation.

GEORGE A. RICHTER. 45  
MILTON O. SCHUR.